

Patented Nov. 9, 1926.

## UNITED STATES PATENT OFFICE.

LESTER KIRSCHBRAUN, OF CHICAGO, ILLINOIS.

## PROCESS OF MAKING WATERPROOF PRODUCTS.

No Drawing.

Application filed January 16, 1925. Serial No. 2,787.

This invention is in part an improvement on my issued Patent No. 1,417,840, dated May 30th, 1922 and in part a continuation of application Serial No. 525,100 filed December 27th, 1921. Heretofore, I have had issued to me U. S. Patent No. 1,536,399 dated May 5th, 1925 and have co-pending application Serial No. 582,303 filed August 16th, 1922, in which a bituminous or pitchy product in an emulsified form or otherwise non-adhesive condition, is mixed with pulp before or during the felting of the pulp on a paper forming apparatus, or the emulsion applied to the surface of the wet web during formation. By means of my prior processes referred to, a paper or other sheet may be formed on paper forming apparatus in which there is incorporated bitumen, which becomes coalesced into continuous films when dry.

More particularly, my prior processes referred to may be carried out as follows:

I make a suitable non-adhesive bituminous emulsion of, for example, water, colloidal clay and asphalt or other bitumen, in which the bitumen forms the internal phase and the water the external phase of the emulsion. This emulsion may be mixed with the fibrous pulp in the usual beater and the mixture flowed over a paper machine to form a web or sheet, or the emulsion applied as a coating to the wet web. As the sheet passes over the driers, the water is removed and the bitumen allowed to coalesce.

Not only may ordinary paper be formed, as, for example, building paper, roofing, flooring or the like, but paper suitable for box board or other forms of containers may be produced.

As is well known to those skilled in the art, the amount of waste paper, either in the form of boxes, containers or otherwise, in the aggregate forms a huge volume. In addition, the broke from paper formed by the process above described, itself constitutes a substantial amount.

The object of the present invention is to re-use the material contained in the old boxes or containers or the broke or otherwise waste paper produced by the above processes and containing asphalt or other pitchy binder, to form new waterproof products. This is accomplished by suitably treating the waste products referred to and re-using them in the beaters, either alone

or mixed with fresh stock, to form such waterproof products.

In re-using such waste materials, the method of treatment will depend considerably upon the amount and character of waterproof material contained in the waste. Where the amount of bituminous material is not too large, effective recovery can be brought about by charging the beaters in the usual way and employing water heated to approximately the melting point of the bituminous material contained in the charge. The effect of the hot water is to soften the bituminous material so that under the action of the beater roll, the fibres become disengaged and freed from contact. It is advantageous in carrying out the beating operation to bring the roll down upon the bed plate to a light brush so as to avoid cutting the fibres and rather separate the matted stock. The beating operation otherwise is carried on in the usual manner until the stock is freed and ready to be used on the machine. If desired, the stock, after sufficient treatment may be washed in the usual washer so as to remove as much of the bituminous matter as has been freed by the beating action from the stock.

When the waste paper is composed of hard stock and where the amount of asphalt is relatively great, the above operation is advantageously supplemented by introducing into the beater a small amount of alkali soda ash, silicate of soda, or equivalent material, which assists the disintegrating action of the beater operation. Where treatment of the above character is employed, there should be added to the stock before running upon the machine, sufficient alum to neutralize the alkali and to precipitate the disengaged asphalted particles upon the fibres. The effect of this latter treatment is to produce an envelope or protective coating of bulky gelatinous precipitate about the asphaltic particles. In any event, however, a desirable feature but not always necessary, is to precipitate or flocculate the asphaltic particles upon the fibres by the use of alum or equivalent flocculating agent, whether alkali is used or not. This renders the material sufficiently non-sticky so that it may be run over the paper machine in combination with other stocks without gumming up the apparatus. When the sheet is formed in the usual way, the water is removed and the

protective coating broken during the drying of the sheet.

Another method of re-using the waste products above referred to is as follows:

- 5 To the asphalted stock in the beaters is added a relatively small amount of oleic acid, sulphonated castor oil, or sulphonic acid salts, such as possess the properties of acting upon and dissolving the asphalt in
- 10 the stock. After a sufficient period of treatment in the beaters with the above agents, an alkali may be added, resulting in the emulsification of the bituminous material and its rapid disengagement from the fibrous stock in the form of discrete particles.
- 15 This treatment renders the recovered asphalt non-adhesive, so that upon subsequent treatment with alum and precipitation upon the fibres, the stock can be run over the paper machine in the usual manner. The amount of the above re-agent will vary with the character of the stock and the amount of asphalt contained therein, but ordinarily about 2% of emulsifying base, will serve to
- 20 carry out the above operation.

In addition to the above substances, it will be understood that other emulsifying bases may be employed, particularly those having the property of miscibility with both asphalt and water.

The distinguishing characteristics of the process described herein, over the process described in my issued United States Patent No. 1,417,840 is that that patent deals primarily with waste saturated felt, which felt was saturated, impregnated or coated with bituminous material, by immersion, after it had been formed into a felted sheet and dried, as is customary in the manufacture of roofing, while the present invention deals primarily with the recovery of waste fibrous stock in which the bituminous waterproofing material with an emulsifying agent was incorporated with the fibrous stock simultaneously with the felting thereof while same was wet.

Such material as is referred to in the present invention, may have bitumen contained throughout the entire body of the sheet, or board, and in quantities varying from that which produce a minor water-repellant action which fully saturates the sheet, or this waste may comprise the product of a multi-cylinder board machine in which only one or more of the plies, preferably the inner plies, contain heavily asphalted stock while the adjoining plies usually four or five, contain untreated or asphaltic stock. In the latter case the recovery takes place in the presence of a largely predominating amount of untreated stock, the asphalt usually comprising less than 20% by weight of the entire sheet. It will be apparent that there is a difference between stock of the character treated by

present invention, and that of waste saturated felt, in that the waste saturated felt always contains a prepondering amount of asphaltic materials usually of a fairly soft nature, whereas the material treated by the present invention presents a wide range of constitution as regards amounts of bitumen present, the nature of the bitumen, and the presence of the emulsifying agent originally incorporated in the sheet.

It has been found in actual practice that the stock prepared in accordance with the present invention from a multi-cylinder board or waste, is particularly adapted for application to the inner plies of a multi-cylinder sheet generally without the addition of fresh stock. This is true for the reason that such stock is generally beaten quite short as a result of the recovery operation, and also on account of its contained asphalt, is "slow" and produces a dense inner ply particularly adaptable for receiving additional quantities of asphalt either in the form of a film application, or in admixture with the stock.

I claim as my invention:

1. A process of recovering waste fibrous products having incorporated therein a bituminous waterproofing binder with a dispersing agent simultaneously with the felting, comprising in subjecting said waterproof fibrous products in an aqueous vehicle to beater action at an elevated temperature approximating the melting point of the binder contained in the waste fibrous stock, causing separation of the fibres precipitating the bituminous material on the separated fibres to render same non-sticky, and felting the stock on a paper machine.

2. A process of recovering waste fibrous products having incorporated therein a bituminous waterproofing binder with a dispersing agent simultaneously with the felting, comprising subjecting said waterproof fibrous products in an aqueous vehicle to beater action at an elevated temperature approximating the melting point of the binder contained in the waste fibrous stock, and adding a flocculating agent to precipitate the binder upon the fibres.

3. A process of recovering waste fibrous products having incorporated therein a bituminous waterproofing binder comprising subjecting said waterproofed fibrous products in an aqueous vehicle to beater action at an elevated temperature approximating the melting point of the binder contained in the fibrous stock causing separation of the fibres from said bituminous material, precipitating the disengaged bitumen on the separated fibres, producing an envelope and felting the stock on a paper machine.

4. A process of recovering waste fibrous products having incorporated therein a bituminous waterproofing binder comprising

subjecting said waterproofed fibrous products in an aqueous vehicle to beater action at an elevated temperature approximating the melting point of the binder contained in the fibrous stock to separate the fibres and bituminous material, adding fresh fibrous stock to the beater precipitating the disengaged bituminous particles on the separated fibres, rendering the mixture non-adhesive and felting the mixture.

5. A process of recovering waste fibrous products having incorporated therein a bi-

tuminous waterproofing binder with a dispersing agent simultaneously with the felting, comprising subjecting said waterproofed fibrous products in an aqueous vehicle to beater action at an elevated temperature approximating the melting point of the binder contained in the fibrous stock, in the presence of an alkali, adding a metallic salt to produce an enveloping coating and felting the stock on a paper machine.

15 20  
LESTER KIRSCHBRAUN.